

## UNITED STATES PATENT OFFICE.

ROBERT ABBOTT HADFIELD, OF SHEFFIELD, ENGLAND.

## METHOD OF TOUGHENING MANGANESE STEEL.

SPECIFICATION forming part of Letters Patent No. 731,450, dated June 23, 1903.

Application filed December 24, 1902. Serial No. 136,484. (No specimens.)

*To all whom it may concern:*

Be it known that I, ROBERT ABBOTT HADFIELD, a subject of the King of Great Britain, residing at Sheffield, county of York, England, have invented an Improvement in Methods of Toughening Manganese Steel, of which the following description is a specification.

My present invention has reference to improvements in the method of toughening manganese steel which forms the subject of my prior patent, No. 572,891.

As the result of costly and exhaustive experiments I have found that exceptional toughness and tenacity can be obtained by the following treatment—that is to say, the manganese steel is put into a heating-furnace the temperature of which is gradually raised, so that heat will be applied very gradually to the steel in order to prevent sudden expansion thereof, this preliminary heating being (as stated in the specification of my before-mentioned patent) conducted at a very slow rate, dependent upon the thickness of the steel, the thicker the steel the slower the rate of heating. Having been slowly heated to a temperature of from 750° to 800° centigrade, (seven hundred and fifty to eight hundred degrees centigrade,) the heating is forthwith expedited, so as to raise the steel as quickly as possible to the temperature at which it is to be plunged in cold water, which temperature, according to my present invention, while varying within certain limits, dependent upon the character of the particular steel and the product required, is not less than 940° centigrade (nine hundred and forty degrees centigrade) or more than 1,125°, (eleven hundred and twenty-five degrees centigrade,) preferably from 980° to 1,050° centigrade (nine hundred and eighty to one thousand and fifty degrees centigrade) in the case of castings and from 940° to 1,000° centigrade (nine hundred and forty to one thousand degrees centigrade) in the case of forged manganese steel.

I find that by treating manganese steel in the manner described the percentage of hardening carbon remaining in the toughened product varies according to the temperature to which the manganese steel was raised previous to its being plunged into cold water, the higher the said temperature the less being the amount of hardening carbon present in the finished product. For example, by

heating different manganese-steel castings, each composed of manganese steel of the same original composition, to 850° centigrade, (eight hundred and fifty degrees centigrade,) 55 900° centigrade, (nine hundred degrees centigrade,) and 1,000° centigrade, (one thousand degrees centigrade,) respectively, the amount of hardening carbon present in the toughened manganese steel was found to be .45 per cent., (decimal four five per cent.,) .36 per cent., (decimal three six per cent.,) and .32 per cent., (decimal three two percent.) 60 The less the amount of hardening carbon present in the finished product the tougher and less hard will be the product, and the greater the amount of hardening product 70 present the harder and less tough will be the product. Consequently it will be seen that by suitably and carefully regulating the temperature to which the manganese steel is raised—as, for example, by a pyrometer—75 the percentage of hardening carbon present in the finished product can also be regulated with considerable accuracy, with the result that toughened manganese steel of a more uniform character and reliable quality can 80 be produced according to this invention than has heretofore been usual.

I claim—

1. The herein-described process of toughening manganese steel, which consists in 85 slowly heating the steel to a temperature from about 750° to about 800° centigrade, and then raising the temperature rapidly to from 940° to 1,125° centigrade, and finally plunging the highly-heated steel in cold water. 90

2. The herein-described process of toughening manganese steel by varying the amount of hardening carbon therein, which consists in slowly heating the steel to a temperature of at least 750° centigrade, and then quickly 95 raising the temperature to at least 940° centigrade, increasing the temperature above said limits the tougher and less hard the desired product, and finally plunging the highly-heated steel in cold water. 100

In testimony whereof I have signed my name to this specification in the presence of two subscribing witnesses.

ROBERT ABBOTT HADFIELD.

Witnesses:

BAIN L. CAMPBELL,  
EDWARD S. ALLSOP.